

## UNITED STATES PATENT OFFICE

TURE ROBERT HAGLUND, OF STOCKHOLM, SWEDEN

## REFRACTORY MATERIAL

No Drawing. Original application filed November 12, 1927, Serial No. 232,947, and in Germany June 4, 1927. Divided and this application filed October 6, 1928. Serial No. 310,917.

This invention relates to a fused refractory material having as essential components oxides of magnesium and aluminum. This application is a division of my co-pending application Serial No. 232,947 of November 12th, 1927. The new product may especially be produced as a slag by reducing oxides or oxide ores in electric furnaces. A typical slag of the new kind has 10 for example the following composition:

|                   | Per cent |
|-------------------|----------|
| Silicic acid      | 11.2     |
| Aluminum oxide    | 34.5     |
| Iron oxide        | 3.0      |
| 15 Titanium oxide | 2.0      |
| Manganese oxide   | 0.4      |
| Chromium oxide    | 21.5     |
| Calcium oxide     | 3.2      |
| Magnesium oxide   | 23.6     |

20 The relation between the contents in the slag of magnesium oxide and aluminum oxide respectively may be varied within very wide limits. However, the magnesium oxide content should be at least 15% and the aluminum oxide content preferably greater than 25%. If no chromium oxide is occurring, the total content of oxides of magnesium and aluminum together with in certain cases occurring titanium should at least amount to 75% of the total oxide content of the slag. The content of silica should be low or less than 15% and suitably below 12%. The content of iron oxides in the slag should be less than 5%.

A considerable amount of chromium oxide has proved to have a very favorable influence upon the chemical resistance of the refractory slag. Said influence is considerable already by 5 to 8%  $\text{Cr}_2\text{O}_3$ . The best results, however, are obtained with a chromium oxide content from about 10 up to about 35 percent. In case of chromium oxide the content of chromium oxide in excess of 5% counted together with oxides of magnesium and aluminum should preferably amount to at least 75% of the total oxide content of the slag.

The new product may be obtained in electric furnace reduction processes either by

selection of the raw materials for that purpose or by adding slag forming admixtures in form of material containing magnesium oxide, aluminum oxide or chromium oxide.

The reduction may for instance be utilized in the production of iron or iron alloys out of iron ores. Such ores contain usually comparatively small quantities of magnesium oxide and aluminum oxide but on the other hand often a considerable content of 55 silicic acid. Most convenient for carrying out the process is to select ores with low or a comparatively low silicic acid content because in such cases it will be easier to adapt the composition of the slag so that a good 60 highly refractory material can be obtained out of it. If however, it is not possible by suitably selecting the raw material to obtain a slag with low silicic acid content special 65 slag forming admixtures are to be used. As 70

slag forming admixtures in the process, magnesite in a burnt or unburnt state and bauxite are used with advantage. If the iron ore contains a high percentage of silicic acid, 75 the same may, however, be decreased to a percentage low enough for obtaining a highly refractory material. This may be done either by reducing a part of the silicic acid so that iron containing silicium is obtained, or by adding magnesite or bauxite with a 80 low content of silicic acid, or by adding a larger quantity of such material that might contain a somewhat higher percentage of silicic acid but still substantially less than 15% of the slag forming oxides in the said 85 admixtures. It is of advantage to regulate the process in such a way that the silicic acid content in the slag is less than 12%, while hereby besides a more refractory material, 90 a substantially increased resistance against chemical influences is achieved. For the rest the proportions between iron ore and slag forming ingredients containing  $\text{MgO}$  or  $\text{Al}_2\text{O}_3$  may be varied within very wide 95 limits. Even iron ores containing titanium may be used in the process. The reduction process is then suitably so carried out that all or a part of the titanic acid in the ore goes into the slag as a component.

The new refractory product may also in the first place be produced in connection with the production of chromium alloys, such as low carbon ferro-chromium. A highly refractory product containing  $\text{Cr}_2\text{O}_3$  may for example be obtained by so adapting the composition of the charging materials in reduction processes for producing ferro-chromium, chromium steel or other chromium alloys, for example by adding magnesite or bauxite or both, that a desired chromium content is received in the slag. It is especially suitable to decrease the total content of silicic acid and ferrous oxide to at the most 15%. The content of magnesium oxide in the slag may partly be replaced, but at the most to one fourth, with calcium oxide. The highly refractory materials may of course also be produced by smelting together materials suitable for the purpose. One may then start either from the simple oxides themselves or from suitable minerals and out of them for example produce a refractory material holding in accordance with the above statements for the main part oxides of chromium, magnesium and aluminum, chromium oxide for example occurring in quantities from a few up to 35% and magnesium oxide from 15% and more. The smelting may be undertaken in tapping furnaces as well as, for example in batch processes, in furnaces of the same kind as ordinarily used in the production of alundum. The received smelt may be directly cast into suitable moulds, whether the same has been obtained in the form of a slag from any metallurgical or other reduction process or if the same has been brought into molten condition by means of other smelting processes. For this purpose it is of advantage that the total content of oxides of iron and silicium be not too low. The same should in such a case not be less than about 5%. Hereby a more fluid slag and a tight slag stone are obtained.

Another way of treating the new refractory material consists in crushing the cooled smelt and using it as a stamp mass or for the manufacture of bricks. As binding agent small quantities of clay substances, sodium silicate, Sorel cement, suitable hydrates, such as those of magnesium, aluminum or chromium, or other binding means may be used.

The new highly refractory material or the articles produced thereof possess besides an extraordinary high refractory ability and a high softening temperature a great chemical resistance. It is for instance especially suitable for use in open hearth furnaces, arches, lining of furnace channels and as material for furnace bottoms.

I claim:—

1. As a new article of manufacture a fused refractory material containing not less than

15% of oxide of magnesium, not less than 5% of oxide of chromium, not less than 75% of oxides of magnesium, aluminum and chromium counted together, and with a content of silica less than 12% and of oxide of iron less than 5%, characterized by high softening temperature and resistance against chemical erosion. 70

2. As a new article of manufacture a fused refractory material containing not less than 5% of oxide of chromium, not less than 15% of oxide of magnesium, not less than 25% of oxide of aluminum, not less than 75% of oxide of magnesium, aluminum and chromium together, and from 5 up to 12% 75 80 of silica.

3. A refractory material having as an essential component particles of a fused refractory material containing from 5 up to 35% of oxide of chromium, not less than 15% of magnesium oxide, not less than 75% of oxides of magnesium, aluminum and chromium counted together, less than 12% 85 90 of silica, less than 5% of iron oxides, and calcium oxide in an amount less than one fourth of the percentage of magnesium oxide.

4. A refractory material having as an essential component particles of a fused refractory material containing not less than 5% of oxide of chromium, not less than 75% 95 of oxides of magnesium, aluminum and chromium counted together, from 5 up to 12% of silica and less than 5% of iron oxides. 100

In testimony whereof I have hereunto set my hand.

TURE ROBERT HAGLUND.

105

110

115

120